# EUROPEAN PATENT APPLICATION

(11) **EP 0 486 939 A1**
(43) Date of publication of application: **27.05.1992**
(21) Application number: 91119387.8
(22) Date of filing: 13.11.1991
(51) Int. Cl.: C21D 8/00, C21D 8/10, B21K 21/04

(54) **Two-pass drawing technique for creating high strength tubing**

(30) Priority: 13.11.1990 US 613076
(71) Applicant: ALLIANT TECHSYSTEMS INC., Edina, Minnesota 55436 (US)
(72) Inventor: Nelson, Stanley R., Minneapolis, MN 55418 (US)
(74) Representative: Altenburg, Udo, Dipl.-Phys.

(57) **Abstract**

A method of producing high performance cartridge cases by processing alloy steels of interest into high strength tubing is disclosed which includes subjecting the annealed alloy steel of interest to at least two passes of drawing in which the total area reduction of each pass is such that the exit temperature of the drawn alloy steel of interest remains below a temperature which will affect austenite to martensite transformation and age hardening the material of interest. The alloy steel of interest is one selected from a group of alloys consisting of metal that undergo phase transformation during work hardening.

## Description

Reference is made to a related application, Serial No. , filed of even date and assigned to the same assignee as the present application. The related application involves an unique alloy steel processing technique for high strength cartridge casings applicable to the same or similar materials.

The present invention identities and defines a process for forming thin-walled, elongated tubing members, particularly of steel or alloy steel, having superior mechanical properties. In particular, the invention is directed to a process for creating very high strength cartridge case tubing bodies which house 20mm to 50mm high velocity projectile assemblies. The invention includes the discovery of a previously unknown and unwanted anisotropic mechanical behavior of the preferred steel material and provides a simple processing solution which elevates the mechanical properties into a functionally acceptable range.

### Cartridge Case Manufacture

The materials commonly employed for high strength cartridge case bodies are 7000 series aluminum alloys and steel, typically a modified medium carbon material. Patent references by Irmann (U.S. Patent 2 220 652) and Rayle, et al. (U.S. Patent 4 041 868) identify basic fabrication techniques associated with aluminum and steel case manufacture, respectively. The case geometry created by those fabrication techniques is compared to that of the current invention in Figures 3A-3C.

Figure 3A corresponds to the Irmann cartridge case shown generally at 20. It includes a head section 21, a generally cylindrical wall section 22 of tapered diameter and a mouth 23 of reduced diameter. While generally cylindrical, the side wall tapers gradually from the head 21 to the more abrupt or necked-down transition at 24. The thickness or gauge of the side wall 22 denoted at 25 also decreases gradually from the head 21 to the mouth 23. The cartridge of Rayle, et al. is similar in geometry and is illustrated generally at 30 in Figure 3B. It includes a head 31, a tapered diameter wall section 32 and a mouth 33 of reduced diameter. The thickness 34 of the wall 32 also decreases from the head 31 to the mouth 33.

The related art, thus, shows dual diameter tapered wall case products for use in a breech housing with matching geometry. Consequently the cartridge case enters and exits the breech from the same end.

The shape required for the cartridge cases of present invention is one of a constant wall thickness right circular cylinder 40, as shown in Figure 3C. This design is required because the gun systems of interest employ a moving breach. In such a design the fired cartridge case housing must exit the breech from the end opposite that through which it entered. This is referred to as a feed-through breech system.

The importance of elasticity in a cartridge case body is well known. Case body expansion during firing must not result in significant permanent set which would otherwise jam the spent case in the breech. The case body designs identified as related art do in fact change shape during firing but their tapered shape match to the tapered breech profile still allows reliable ejection. Consequently, earlier processes pay no attention to definition and control of circumferential mechanical properties, whereas this parameter is the key feature of the current invention for feed-through breech systems.

### Alloy Selection

The cartridges employing the current invention case body are usually fired from land vehicles with crew members in close proximity to the gun and its breech system. Consequently, aluminum alloy case material is not employed as case fracture during firing results in severe aluminum melt down which does considerable breech damage and puts the vehicle crew in danger of injury from its own ammunition.

The 20mm to 50mm size ammunition family is the primary class of interest with respect to the present invention. A 17-7PH stainless steel is the preferred material of construction. This material, when properly processed, can provide circumferential yield strength in excess of 170,000 psi while retaining typically 8 percent elongation which is sufficient for cartridge assembly and functional application in the class of interest.

Rayle, et al., cited above, identify a modified medium carbon steel case capable of being heat treated to a range of 150,000 psi to 215,000 psi tensile strength, protiably in the longitudinal direction. The 215,000 psi tensile strength value will provide approximately 182,000 psi yield strength which would be in the range of interest for the current invention. However, these high strength values identified by Rayle, et al. are achieved by severe brine quenching from 1600 to 1700^{o}F followed by tempering. Such a heat-treat process, however, is known to create severe distortion and uncontrolled volume expansion of such a magnitude that they could not be tolerated for fabrication at thin wall right circular cylinder case bodies which are used in feed-through breech systems.

While other materials can be used, as discussed in detail below, 17-7PH stainless steel is preferred for most applications of the invention because it can provide the desired strength and is well known to be isotropic (i.e., mechanical properties of equal value in all directions). The isotropic nature of the material is demonstrated for sheet stock in Figure 4A. As a semi-austenitic steel, 17-7PH can be roll reduced in thickness up to at least 45 percent area reduction and retain its isotropy when age hardened at 900^{o}F.

The drawn welded 17-7PH tubing, conventionally heat treated to be high strength cartridge case stock, however, had been found to exhibit decidedly asymmetric yield strength properties. Although the material behaves according to published data with respect to dimensional predictability, strength figures do not follow the pattern. The yield strength in the circumferential direction has been found to be much lower than that in a longitudinal direction, due to the presence of a mechanical property anisotropy which is totally unexpected. This results in the stock being unacceptably weak as depicted in the left hand portion of Figure 5 where the hardened tubing has a circumferential yield strength of only 157,000 psi.

A need has existed to substantially improve the performance of this and similar materials fabricated into cartridge cases and other high performance tubing parts by increasing the circumferential yield strength to an acceptable level as for the applications discussed. Accordingly, it is a primary object of the present invention to provide a heat treating process by which very high strength, high alloy steel tubing can be created which exhibits substantially increased circumferential yield strength characteristics after cold working.

It is a further object of the present invention to accomplish substantially increased tensile and yield strength characteristics in alloy steel tubing utilizing a relatively inexpensive process.

### SUMMARY OF THE INVENTION

The present invention provides a process by which alloy steel tubing can be cold worked (definitions and some discussion of metal processing are presented below) in a manner which results in very high tensile and yield strength values. The process of the invention involves the discovery that, contrary to conventional cold working practice, multiple pass tube drawing techniques which achieve essentially the same total area reduction as that of a maximized single pass draw can result in much higher performance mechanical properties.

A multi-pass plug draw process is utilized to achieve the same overall area reduction rather than accomplishing the entire reduction in one draw. This greatly reduces the work or energy input per pass to which the tube is subjected and this, in turn, reduces the exit metal temperature reached by the material during the drawing process. The exit metal temperatures achieved by a reduction of about 40 percent utilizing a two-pass plug draw of substantially equal reduction per pass was found to be about 140^{o}F for each pass which, it has been found, doss not retard austenite to martensite transformation and thus allows much higher strengths to be achieved by later age hardening. It is believed that exit metal temperatures below about 170^{o}F should be satisfactory. Higher exit metal temperature, such as achieved using a single pass plug draw, appears to retard further strengthening during age hardening at 900^{o}F.

In the preferred embodiment, the stock stainless steal tubing received is subjected to several processing steps. First, the material is conditioned at a temperature in the range of about 1950^{o}F in a standard preconditioning or annealing step in which it is held at that temperature for about 15 minutes and allowed to cool to room temperature. Thereafter, the tubing is subjected to two plug draw steps in which approximately the same area reduction is achieved. A total area reduction of about forty percent (40%) is realized by the two-pass plug draw. This may be followed by a sink draw step. The material is then subjected to age hardening for about one-half to one hour at approximately 900^{o}F.

The preferred embodiment requires but two passes to achieve the reduction and strength requirements necessary for high strength cartridge applications; however, it is believed that processes using additional passes would be applicable. The exit metal temperature should be kept below that which retards austenite to martensite transformation.

The process can be used with any metal alloys that undergo phase transformation during work hardening to increase strength properties, including austenitic or semi-austenitic stainless steels. More specifically, type 302, 304, 316, PH15-7MO AND 17-7PH alloy stainless steels are examples of such materials. The preferred material is 17-7PH stainless steel.

The process is described with respect to drawn tubing. However, it is also applicable to other drawn materials including steel wire and steel springs when such are made from appropriate materials.

In the drawings, wherein like numerals are utilized to designate like parts throughout the same:
Figure 1 is a fragmentary view, partially in section, that illustrates a plug drawing apparatus which can be used in accordance with the process of the invention;
Figure 2 is a view similar to that of Figure 1 illustrating a sink draw apparatus;
Figures 3A and 3B illustrate prior art cartridge cases;
Figure 3C illustrates a section of cartridge casing stock fabricated in accordance with the invention;
Figure 4A represents theoretical or handbook values of certain mechanical properties of the metal of the preferred embodiment;
Figure 4B is a key for Figure 4A;
Figure 5A represents a comparison of actual mechanical properties versus test direction achieved utilizing single and two-pass draws; and
Figures 5B and 5C are keys for Figure 5A.

The following description illustrates the principles of the present invention with respect to one or more specific alloy steels. Prior to discussing specific details of the invention process itself, however, it is believed that some discussion of metal processing would be helpful.

### Metal Structure

Iron and iron alloys exhibit several crystal lattice forms with respect to the position of the iron atoms in the structure Austenite is one form defined as a solid solution of one or more elements in face-centered cubic iron. Although it may include other elements such as nickel and/or chromium, the solute is generally assumed to be carbon. Martensite, on the other hand, is defined as a metastable phase of steel formed by the transformation of austenite which occurs below an initial transition temperature known as the M_{S} temperature. Martensite is an interstitial supersaturated solid solution of carbon and iron which has a body-centered tetragonal lattice. Its microstructure is characterized by an acicular or needle-like pattern. Transformation from the face-centered to the body-centered form is normally accompanied by a volume expansion of the material.

### Processing

Mechanical processes applied to ambient or near ambient temperature metals, of course, are known as cold working. Cold working may be defined as deforming metal plastically at a temperature lower than its recrystallization temperature. The recrystallization temperature, in turn, can be defined as the approximate minimum elevated temperature at which complete formation of a new strain-free grain structure from that existing after cold working occurs within a specified time. Cold working of many steels greatly increases the tensile and yield strengths of the material and very high tensile and yield strengths are desirable in high performance cartridge applications because of the tremendous momentary heat and pressure generated during firing.

Cold working of the tubing associated with the manufacture of cartridge cases may include one or more cold draw steps to achieve the desired diameter and wall thickness dimensions. This usually includes one or more plug draw steps which may be followed by sink drawing.

In the plug drawing operation, the tubing is pulled through a shaping die which defines the outside dimension in conjunction with a stationary mandrel having a plug located adjacent the opening in the die such that the die and plug cooperate to determine the wall thickness of the tube being drawn. One end of the mandrel is a rod fixed to a support beyond the end of the tube being drawn and the other end of the rod is connected to the plug such that the plug is supported by the rod and is held stationary relative to the motion of the tube over the plug between the plug and the die. The geometry of the plug is such that the combination of stresses involved holds the plug in the proper concentric position. The results in terms of inside diameter, surface condition and wall thickness tolerances are of such quality that the operation may be used for a final pass to a finished size. Normally area reductions of up to about forty percent (40%) can be accomplished by a single plug draw operation.

Sink drawing involves pulling the tube through a die formed in the desired shape of the outside diameter without any internal support or plug. Sink drawing may be used after plug drawing for the final adjustment of outside sizing with or without any corresponding change in wall thickness and normally produces an article suitable for final finishing processes.

Prior to drawing it is necessary for the material to be made rather uniformly soft and ductile; therefore, it is normal to subject the metal or metal alloy material to a standard conditioning or annealing step in which the material is held at a suitable elevated temperature for a short time and allowed to cool to ambient. In the case of materials of the class for which the present invention best applies, such as austenitic stainless steels, this is known as the austenitic conditioning temperature and is between about 1850^{o}F and 2000^{o}F.

One type of cold working device is illustrated in the fragmentary view of Figure 1 which shows the metal working portion of a plug draw machine partially in section. The device includes a stationary rod member 11 which supports or carries a stationary, internal diameter defining plug member 12 positioned in the tube of interest 15 prior to drawing. The plug member 12 cooperates with an external die 13 mounted on a structural member 14 to determine the thickness and diameter of the tube after the drawing operation. Prior to the drawing operation, one end of the tube 15 is reduced or pointed as by swaging at 16 to facilitate its entry into the opening in the die member 13.

In operation, the plug member 12 with retaining rod 11 are inserted into the unswaged open-end 17 of a section of tubing and mounted in a manner such as the rod 11 is fixed in place relative to the motion of the tube 15 during the drawing operation. A member 18 pulls the member 15 through the die 13 with the plug 12 positioned inside the die so as to produce the desired inside diameter and wall thickness in the drawn tube 19. Geometry of the plug 12 is normally such that a combination of stresses holds the plug in the proper centered position with respect to the tube.

Depending on the hardness of the material, a great deal of stress is generated during the drawing operation in which the member 15 is pulled through the die past the plug in the reduction operation. It will be appreciated that the amount of stress, and therefore heat, which is generated during the drawing operation increased with the amount of area reduction achieved. A plug draw which achieves a 40% area reduction results in a drawing exit metal temperature much higher than a drawing pass which achieves a reduction of 20% or less, for example. In accordance with the present invention, it has been found that with room temperature material drawing passes in which the amount of reduction is less than or equal to about 20% based on the entry material diameter and thickness generally produce an exit metal temperature low enough (≦ 140^{o}F) such that the further strengthening of the material during subsequent age hardening is essentially not adversely affected.

Figure 2 depicts a sink drawing device which is generally utilized for minor, final dimensional changes. Sink drawing is accomplished by pulling the tube 15 through a die 20 without internal support, reducing the outside diameter and inside diameter of the tubing at the same time. This operation may be accompanied by a slight wall thickening, but depending on such factors as size and die contour, the wall thickness may remain unchanged. Sinking is often performed as a final sizing operation after other forms of drawing have accomplished the great majority of the cold reduction.

### Tube Making Process

The process of the present invention involves the modification of one important step in the basic tube drawing procedure to create the desired properties in the cartridge case body material. The process normally consists of a single plug draw of previously softened (solution annealed) 17-7PH steel to final wall thickness and diameter. A sink draw finishing step may also be employed if desired to precisely adjust the finished diameter. The discovery of the invention involves a change in the drawing process which will be described next.

As discussed above, when steel is transformed from austenite to martensite by either heat treatment or work hardening a significant volume expansion occurs. This phenomena must be neutralized during fabrication of high strength case bodies to control the diameter of the end item. In the cold working process, the 17-7PH stainless steel transforms from austenite to martensite during the cold working of the plug draw. The relatively large changes in diameter and wall thickness during this operation easily compensate for the volume expansion. Since cold worked 17-7PH stainless steel undergoes a modest and predictable shrinkage when ago hardened it logically follows that this tubular product only need be cut to length then age hardened after drawing to provide desired isotropic mechanical properties and achieve desired dimensional detail.

This assumption proved to be true for the dimensional detail but the resulting yield strength in the circumferential direction was found to be much lower than desired due to the totally unexpected presence of mechanical property anisotropy. The following examples will illustrate this finding and show how the modified cold working tube draw process of the invention increases resultant circumferential yield strength to an acceptable level.

### Example 1

This example pertains to a 30mm size cartridge product test series. In order for the 30mm size case of the example to function without sticking a 170,000 psi yield strength must be created in the circumferential direction. After annealing, a 37 percent area reduction single pass plug draw was employed. Tensile testing in the longitudinal and circumferential direction after age hardening gave results quite contrary to established theory. Anisotropy (mechanical properties significantly lower in the circumferential direction) was found. As depicted in Figure 5, the resultant typical yield strength of only 157,000 psi was achieved, well below the required minimum.

### Example 2

Material from the same treatment lot as Example 1 was plug draw processed using two draws instead of one to achieve a similar area reduction (i.e., the final plug draw was through the same die as used in Example 1). Subsequent age hardening produced a typical yield strength Of 184,000 psi in the circumferential direction. Although anisotropy was still evident the yield strength was substantially increased to a satisfactory level which was later verified in cartridge firing tests.

The following additional example sets represent test runs utilizing material from the same heat lot of sheet alloy stainless steel which was uniformly subjected to a standardizing step at 1950^{o}F.
17-7 PH stainless steel tubing 2.121" diameter x .019" thick wall:

As can be seen from the comparison of Examples 1 and 3 with Examples 2 and 4, both the longitudinal and circumferential tensile strength and yield strength are greatly increased utilizing a two-pass cold reduction process.

Figures 4A and 4B represent available textbook or handbook data (Armco Steel Handbook, 1975) concerning rolled reduction and age hardening with respect to the same 17-7 PH stainless steel exemplified in the Examples. As can be seen from Figure 4A, the established theory indicates that directionally cold worked (rolled) 17-7 PH sheet stock undergoes a substantial increase in both tensile and yield strength upon subsequent age hardening at 900^{o}F for one hour. It should be noted that the handbook values for 35% and 40% reduction in Figure 4 far exceed those of Examples 1 and 3 which utilized a single cold draw pass to achieve 37.6% area reduction. The substantially anisotropic nature of the strength properties evidenced by the Examples also are not shown in the directionally cold worked rolled 17-7 PH sheet stock data from the handbook. It is only after utilizing the two-pass cold plug draw area reduction technique of the invention that the tensile and yield strengths achieved approach those given for rolled and hardened material in Figure 4.

The mechanism of change is created by a difference in exit metal temperature from the plug draw die. The two plug draw procedure was measured for exit metal temperature and found to average 140^{o}F. Although a single pass plug draw was not measured it is expected to be well above 200^{o}F. The elevated exit metal temperature retarded austenite to martensite transformation creating a lower yield strength in the as-drawn and subsequently age hardened material. These factors are shown in the mechanical property summary of Figure 5. The single pass plug draw gave only 89,000 psi circumferential yield strength whereas the two pass plug draw gave 106,000 psi yield strength. An as-drawn circumferential yield strength of 96,000 psi apparently is required to guarantee an as-aged yield strength of 170,000 psi.

Figure 5 further illustrates the improvement achievable by utilizing the two-pass redraw process in accordance with the invention. It should be noticed that whereas the two-step or multiple step redraw process of the invention greatly increases both the tensile strength and the yield strength of the material, the anisotropic nature remains. For most applications, if the transverse yield strength is sufficient, the anisotropic nature of the mechanical properties of the material becomes less important.

The present invention identifies anisotropy in a 17-7PH stainless steel previously believed to be isotropic and emphasizes the importance of exit metal temperature control in tube plug drawing in order to achieve the high mechanical properties required for cartridge case body components. The two pass redraw step is just one means of controlling exit metal temperature. Since lower temperature should result in still higher mechanical properties, such approaches as water cooled dies and chilled feedstock could be employed.

The lower reduction percentages for each draw pass also allow better diameter dimensional control because the metal expansion during drawing is more uniform and predictable. In addition, there is a higher yield of usable material because lower reduction percentages can be utilized to achieve a given high strength requirement. It has also been found that the two-pass draw technique yields tubing in which better control and consistency is achieved with respect to final part dimensions as only modest shrinkage occurs during the subsequent age hardening treatment.

This invention has been described in this application in considerable detail in order to comply with the Patent Statutes and to provide those skilled in the art with the information needed to apply the novel principles and to construct and use such specialized components as are required. However, it is to be further understood that the invention can be carried out by specifically different equipment and devices and that various modifications can be accomplished without departing from the scope of the invention itself.

For example, these discoveries, of course, are not limited to 17-7PH stainless steel or to cartridge case body material. any metal which undergoes phase transformation during work hardening is a candidate. The 302, 304, 316 and PH15-7MO stainless steels are examples of other materials that fall in this class. Other sizes of pressure tubing or deep drawn products could benefit from this discovery. In addition, wire products of such an application of stainless steel material for spring applications could benefit materially.

## Claims

1. A method of processing metal materials of interest into high strength forms comprising the steps of:
annealing the metal of interest at a temperature and for a time sufficient to standardize and soften the material for drawing;
subjecting the metal material of interest to drawing in which the total area reduction of each pass is such that the exit temperature of the drawn alloy steel of interest does not exceed a temperature that will affect subsequent age hardening;
age hardening the metal of interest by heating it to a temperature sufficient to age harden it for a desired time; and
wherein the metal of interest is one selected from a group of alloys consisting of metals that undergo phase transformation during work hardening.

2. A method of producing high performance cartridge cases by processing alloy steel material of interest into high strength tubing comprising the steps of:
austenitic conditioning of the alloy steel material of interest at a temperature and for a time sufficient to standardize the material for drawing;
subjecting the alloy steel material of interest to at least two passes of drawing in which the total area reduction of each pass is such that the exit temperature of the drawn alloy steel of interest does not exceed about 170^{o}F;
age hardening the alloy steel material of interest by heating it to a temperature sufficient to age harden it for a desired time; and
wherein the alloy steel of interest is one selected from a group of alloys consisting of steel alloys that undergo phase transformation during work hardening.

3. The method of claim 2 wherein each pass of the draw results in a reduction of approximately 20% or less.

4. The method of claim 2 wherein the age hardening step is accomplished at approximately 900^{o}F for about one hour, followed by air cooling.

5. The method of claim 3 wherein the age hardening step is accomplished at approximately 900^{o}F for about one hour, followed by air cooling.

6. The method of claim 2 wherein the exit temperature of the draw is less than or equal to 140^{o}F.

7. The method of claim 3 wherein the exit temperature of the drab is less than or equal to 140^{o}F.

8. The method of claim 4 wherein the exit temperature of the draw is less than or equal to 140^{o}F.

9. The method of claim 5 wherein the exit temperature of the draw is less than or equal to 140^{o}F.

10. The method of claim 9 therein the material of interest is selected from the 302, 304, 316, PH15-7MO and 17-7PH stainless steels.

11. The method of claim 9 wherein the material of interest is 17-7PH stainless steel.

12. A method of producing high performance cartridge cases by processing alloy steel materials of interest into high strength tubing comprising the steps of:
annealing the alloy steel of interest at a temperature of about 1950^{o}F and for a time sufficient to standardize the material for drawing and cooling the material substantially to ambient;
subjecting the alloy steel material of interest to at least two passes of drawing in which the total area reduction of each pass is such that the exit temperature of the drawn alloy steel of interest does not exceed about 140^{o}F;
age hardening the alloy steel material of interest by heating it to a temperature of about 900^{o}F for about one-half to one hour; and
wherein the alloy steel material of interest is one selected from a group of alloys consisting of steel alloys that undergo phase transformation during work hardening selected from the group consisting of the 302, 304, 316, PH15-7MO and 17-7PH stainless steels.

13. The method of claim 11 wherein the alloy steel material of interest is 17-7PH stainless steel.

14. A method of processing alloy steel tubing to improve circumferential mechanical properties in high strength forms comprising steps as follows:
annealing the alloy steel tubing at a temperature and for a time sufficient to standardize and soften the material for drawing;
subjecting the alloy steel tubing to a drawing operation of one or more passes in which total energy input per pass is such that the drawn alloy steel exit temperature does not exceed a temperature that will affect subsequent age hardening;
age hardening the alloy steel tubing by heating it to a temperature and for a period of time sufficient to accomplish age hardening;
wherein the alloy steel is one selected from a group consisting of those steel alloys that undergo phase transformation during work hardening.

15. The method of claim 29 wherein the age hardening step is accomplished at approximately 900^{o}F for a period of about one hour or less, followed by air cooling.

16. The method of claim 29 wherein the exit temperature of the drawn alloy steel does not exceed 170^{o}F.

17. The method of claim 29 wherein the total reduction of the drawing operation is about 40%.

18. The method of claim 31 wherein the total reduction of the drawing operation is about 20% per pass and the number of passes in the drawing operation is two.

19. The method of claim 30 wherein the exit temperature of the drawn alloy steel does not exceed 170^{o}F.

20. The method of claim 30 wherein the total reduction of the drawing operation is about 20% per pass and the number of passes in the drawing operation is two.

21. A method of producing high strength, high performance cartridge cases by processing alloy steel tubing to improve circumferential mechanical properties comprising steps as follows:
austenitic conditioning the tubing at a temperature and for a time sufficient to standardize the alloy steel tubing material for drawing;
subjecting the tubing to a drawing operation of one or more passes in which the drawn alloy steel exit temperature does not exceed about 170^{o}F;
age hardening the tubing by heating it to a sufficient temperature for a time sufficient to accomplish age hardening;
wherein the alloy steel is one selected from a group consisting of alloy steels that undergo phase transformation during work hardening.

22. The method of claim 36 wherein the drawing operation consists of at least two passes each resulting in a reduction of approximately 20% or less.

23. The method of claim 36 wherein the age hardening step is accomplished at approximately 900^{o}F for a period of about one hour or less, followed by air cooling.

24. The method of claim 36 wherein the alloy steel is selected from 302, 304, 315, PH15-7MO and 17-7PH stainless steels.

25. The method of claim 38 wherein the alloy steel is selected from 302, 304, 316, PH15-7MO and 17-7PH stainless steels.

26. The method of claim 38 wherein the alloy steel is 17-7PH stainless steel.

27. A method of producing high performance precision cartridge cases by increasing circumferential yield strength of high strength alloy steel tubing comprising steps as follows:
annealing the alloy steel at a temperature of about 1950^{o}F and for a time sufficient to standardize the alloy steel for drawing and cooling the material substantially to ambient;
subjecting the alloy steel material of interest to at least two passes of drawing in which the area reduction of each pass is less than or equal to 20% and in which energy input per pass is such that the alloy steel exit temperature does not exceed about 170^{o}F;
age hardening the alloy steel by heating it to a temperature of about 900^{o}F for about one-half to one hour;
wherein the alloy steel is one selected from a group of alloys that undergo phase transformation during work hardening consisting of 302, 304, 316, PH15-7MO and 17-7PH stainless steels.

28. The method of claim 42 wherein the alloy steel material is 17-7PH stainless steel.
